# NEW EUROPEAN PATENT SPECIFICATION

(11) **EP 3 164 524 B2**
(45) Date of publication and mention of the opposition decision: **03.09.2025**
(45) Mention of the grant of the patent: 30.10.2019
(21) Application number: 15728541.2
(22) Date of filing: 12.06.2015
(51) Int. Cl.: C22C 21/00, C22C 21/02

(54) **ALUMINIUM ALLOY FOR USE IN THE BUILDING INDUSTRY**
ALUMINIUMLEGIERUNG ZUR VERWENDUNG IN DER BAUINDUSTRIE
ALLIAGE D'ALUMINIUM DESTINÉ À ÊTRE UTILISÉ DANS L'INDUSTRIE DU BÂTIMENT

(30) Priority: 04.07.2014 EP 14175706
(43) Date of publication of application: 10.05.2017
(73) Proprietor: Novelis Koblenz GmbH, 56070 Koblenz (DE)
(72) Inventor: KIRKHAM, Steven, 56235 Ransbach-Baumbach (DE); JACOBY, Bernd, 65553 Limburg (DE)
(74) Representative: Weickmann & Weickmann PartmbB
(86) International application number: PCT/EP2015/063203
(87) International publication number: WO 2016/000937

(56) References cited:
- EP-A1- 0 300 927
- EP-A1- 1 386 975
- EP-A1- 1 484 420
- EP-A1- 1 484 421
- WO-A1-97/46726
- WO-A2-01/36697
- DE-A1- 19 938 995
- FR-A1- 2 855 833
- JP-A- 2007 131 881
- JP-A- 2010 168 632
- JP-A- H04 371 368
- JP-A- H06 264 171
- US-A- 4 431 463
- US-A1- 2004 062 946
- « bordereau de commande N° 005961 »
- « deuxième page d’une facture du 26/08/2010 correspondant à la commande N° 005961 (colis N° 1405088) »
- « certificat de réception et avis d’expédition du 26/08/2010 (colis N° 1405088) »
- « bon de livraison correspondant à la facture précédente et à la commande N° 005961 (colis N° 1405088) »
- « résumé de la société MIRALU »
- « exemple de réalisation architecturale livrée en 2013 avec des produits MIRALU »
- « bordereau de commande N° 005033 »
- « facture du 19/01/2010 correspondant à la commande N°005033 (colis N° 1363475, 1363477 et 1363481) »
- « certificat de réception et avis d’expédition du 01/03/2010 (colis N° 1363475, 1363477 et 1363481) »
- « bon de livraison correspondant à la facture précédente et à la commande N° 005033 (colis N° 1363475, 1363477 et 1363481) »

## Description

### FIELD OF THE INVENTION

The invention relates to a rolled Al-Si-Mg-Mn alloy sheet product. The sheet product is ideally used for outdoor use in the building industry, for example in the form of trapezoidal sheet.

### BACKGROUND TO THE INVENTION

Some aluminium alloy sheet products in the art for use in the building industry include:
The AA4017 alloy registered with the Aluminium Association in 1995 and consisting of, in wt.%:

| | |
|---|---|
| Si | 0.6 - 1.6 |
| Fe | up to 0.7 |
| Cu | 0.10 - 0.50 |
| Mn | 0.6 - 1.2 |
| Mg | 0.10 - 0.50 |
| Zn | up to 0.20, |

others and unavoidable impurities, each 0.05% max, total 0.15%, remainder aluminium.

Each of European patent document EP-1484420-A1 and EP-1484421-A1 disclose an aluminium alloy product in the form of a sheet or extrusion having a composition of, in wt.%:

| | |
|---|---|
| Si | 1.2 - 2.2, preferably 1.4 - 2, |
| Fe | < 1.5, preferably < 0.7, |
| Cu | 0.2 - 0.8, preferably 0.3 - 0.5, |
| Mn | 0.6 - 1.5, preferably 0.9 - 1.2, |
| Mg | < 0.20, preferably < 0.15, |
| Zn | < 0.5 |
| Ti | < 0.10, |

remainder aluminium and unavoidable impurities.

### DESCRITION OF THE INVENTION

As will be appreciated herein below, except as otherwise indicated, aluminium alloy designations and temper designations refer to the Aluminium Association designations in Aluminium Standards and Data and the Registration Records, as published by the Aluminium Association in 2014 and are well known to the person skilled in the art.

For any description of alloy compositions or preferred alloy compositions, all references to percentages are by weight percent unless otherwise indicated.

For this invention the term "sheet" or "sheet product" refers to a rolled product form in the gauge range of 0.2 to 3 mm in thickness at final gauge.

It is an object of the invention to provide a rolled Al-Si-Mg-Mn alloy sheet product for outdoor use in the building industry providing a balance of strength, corrosion resistance and good formability.

This and other objects and further advantages are met or exceeded by the present invention and providing a rolled aluminium alloy sheet product for outdoor use in the building industry, wherein the aluminium alloy has the following composition, in wt.%:

| | |
|---|---|
| Si | 1.10 - 1.6 |
| Mg | 0.25 - 0.40 |
| Mn | 0.6 - 1.6 |
| Cu | 0.10 - 0.6 |
| Fe | 0.05 - 0.7 |
| Ti | 0.05 - 0.20 |
| Zn | up to 0.4, |

others and unavoidable impurities, each 0.05% max, total 0.25%, balance aluminium.

The rolled aluminium alloy sheet product according to this invention provides a good balance in strength, improved corrosion resistance and good formability, in particular good roll formability. A further advantage of the rolled aluminium alloy sheet product is that it can absorb substantial amounts of Si-containing brazing sheet scrap material originating from the industrial scale production of brazing sheet material.

In an embodiment of the aluminium alloy the Mn-content is at least 0.70%, and preferably at least 0.75%. A preferred upper-limit for the Mn-content at most 1.4% and more preferably at most 1.20%.

In an embodiment of the aluminium alloy the Cu-content is at least 0.15%. The Cu-content is preferably at most 0.5%. In an embodiment the Cu-content is at most 0.4%, and preferably at most 0.35%.

In an embodiment of the aluminium alloy the Fe-content is at least 0.10%. The Fe-content is most 0.7%, and preferably is at most 0.45%.

Zn can be tolerated to substantial levels as an impurity element or can be added purposively. However, in an embodiment of the aluminium alloy the Zn-content is at most 0.25%, and preferably at most 0.20%. In a further embodiment the Zn-content is at most 0.10%, and more preferably at most 0.07%, such that the aluminium alloy is substantially free from Zn.

In the aluminium alloy the Mg-content is least 0.25% to increase the strength and formability of the sheet product. The upper-limit for the Mg-content is 0.40%.

In the aluminium alloy the Si-content is at least 1.10% to increase the strength and formability of the sheet product. In an embodiment the Si-content is at least 1.20%. A preferred upper-limit for the Si-content is 1.50%, and preferably 1.45%.

The Ti is purposively added to the aluminium alloy in a range of 0.05% to 0.20% to enhance the strength and the corrosion resistance, in particular the resistance against pitting corrosion is improved making the sheet product ideally suitable for outdoor use in amongst others the building industry. A preferred lower limit for the Ti-content is 0.07%, and more preferably 0.08%. A preferred upper limit for the Ti-content is 0.17%, preferably 0.15%, and more preferably 0.14%.

Zr is preferably not added to the aluminium alloy of the invention, but can be present as an unavoidable impurity element at a level of <0.05%, and preferably <0.03%, such that the aluminium alloy is substantially free from Zr.

Cr is preferably not added to the aluminium alloy of the invention, but can be present as an unavoidable impurity element at a level of <0.05%, and preferably <0.03%, such that the aluminium alloy is substantially free from Cr.

For the purpose of this invention the aluminium alloy sheet product is a bare sheet product, meaning that on either side it is devoid of any metallic layer(s) covering substantial parts of the sheet product. Such metallic layer(s) are commonly applied by roll bonding or casting techniques for in amongst others brazing sheet products in order to enhance the corrosion performance by providing sacrificial protection to the core alloy or to provide a filler metal, typically an AlSi alloy, for the brazing operation. Such metallic layer(s) have typically a thickness of 4% to up to 15% or more of the total product thickness should the aluminium alloy product have been clad on one or both sides.

The aluminium alloy sheet product can be provided however with a very thin conversion coating to enhance for example the adhesion of any applied organic coating layer, e.g. a paint layer or lacquer.

The aluminium alloy sheet product can be provided with a textured surface structure via sheet metal embossing to provide an attractive surface appearance in the use for building applications such as façade and roof structures.

The aluminium alloy sheet product can be provided in an O-temper or an H-temper, in particular a temper selected from the group of H12, H14, H16, H18, H22, H26 temper.

In a further aspect of the invention it relates to the use, or to a method of use, of the rolled aluminium alloy sheet product according to this invention for outdoor use in the building industry, signposting or decoration. Preferred examples for use in the building industry are façade structures or façade panels, garage doors and metal standing seam roofs. Such applications typically comprise folded or roll formed structures, which may take benefit from the good formability and corrosion resistance of the sheet product in accordance with this invention. A preferred embodiment of the sheet product concerns its use as trapezoidal sheet.

## Claims

1. A rolled aluminium alloy sheet product for outdoor use in the building industry, wherein the aluminium alloy has the following composition, in wt.%:
| | |
|---|---|
| Si | 1.10 - 1.6 |
| Mg | 0.25 - 0.40 |
| Mn | 0.6 - 1.6 |
| Cu | 0.10 - 0.6 |
| Fe | 0.05 - 0.7 |
| Ti | 0.05 - 0.20 |
| Zn | up to 0.4, |
others and unavoidable impurities, each 0.05% max, total 0.25%, balance aluminium.

2. A rolled sheet product according to claim 1, wherein the Mn content is at least 0.70%, and preferably at least 0.75%.

3. A rolled sheet product according to claim 1 or 2, wherein the Mn content is at most 1.4%, and preferably at most 1.20%.

4. A rolled sheet product according to any one of claim 1 to 3, wherein the Cu-content is at least 0.15%, and preferably at most 0.5%, and more preferably at most 0.4%.

5. A rolled sheet product according to any one of claims 1 to 4, wherein the Zn-content is at most 0.25%, and preferably at most 0.20%.

6. A rolled sheet product according to any one of claims 1 to 5, wherein the Ti-content is at least 0.07%, and preferably at least 0.08%.

7. A rolled sheet product according to any one of claims 1 to 6, wherein the Ti content is at most 0.17%, and preferably at most 0.15%.

8. A rolled sheet product according to any one of claims 1 to 7, wherein the Si-content is at most 1.50%, and more preferably at most 1.45%.

9. A rolled sheet product according to any one of claims 1 to 8, wherein the sheet product is devoid of any metallic clad layers.

10. A rolled sheet product according to any one of claims 1 to 9, wherein the sheet product is provided with an organic coating.

11. A rolled sheet product according to any one of claims 1 to 9, wherein the sheet product is provided with a surface structure via sheet metal embossing.

12. A rolled sheet product according to any one of claims 1 to 11 in the form of trapezoidal sheet.

13. Use of an aluminium alloy according to any one of claims 1 to 12 for outdoor use in the building industry, signposting or decoration.

14. Use of an aluminium alloy according to any one of claims 1 to 12 in the form a trapezoidal sheet for outdoor use in the building industry.

## Patentansprüche

1. Walzblechprodukt aus Aluminiumlegierung zur Verwendung im Außenbereich in der Bauindustrie, wobei die Aluminiumlegierung in Gew.-% die folgende Zusammensetzung hat:
| | |
|---|---|
| Si | 1.10 - 1.6 |
| Mg | 0.25 - 0.40 |
| Mn | 0.6 - 1.6 |
| Cu | 0.10 - 0.6 |
| Fe | 0.05 - 0.7 |
| Ti | 0.05 - 0.20 |
| Zn | up to 0.4, |
andere und unvermeidliche Verunreinigungen, je 0,05% max, gesamt 0,25%, Rest Aluminium.

2. Walzblechprodukt nach Anspruch 1, wobei der Mn-Gehalt mindestens 0,70%, und vorzugsweise mindestens 0,75% beträgt.

3. Walzblechprodukt nach Anspruch 1 oder 2, wobei der Mn-Gehalt höchstens 1,4%, und vorzugsweise höchstens 1,20% beträgt.

4. Walzblechprodukt nach einem der Ansprüche 1 bis 3, wobei der Cu-Gehalt mindestens 0,15%, und vorzugsweise höchstens 0,5%, und noch bevorzugter höchstens 0,4% beträgt.

5. Walzblechprodukt nach einem der Ansprüche 1 bis 4, wobei der Zn-Gehalt höchstens 0,25%, und vorzugsweise höchstens 0,20% beträgt.

6. Walzblechprodukt nach einem der Ansprüche 1 bis 5, wobei der Ti-Gehalt mindestens 0,07%, und vorzugsweise mindestens 0,08% beträgt.

7. Walzblechprodukt nach einem der Ansprüche 1 bis 6, wobei der Ti-Gehalt höchstens 0,17%, und vorzugsweise höchstens 0,15% beträgt.

8. Walzblechprodukt nach einem der Ansprüche 1 bis 7, wobei der Si-Gehalt höchstens 1,50% und noch bevorzugter höchstens 1,45% beträgt.

9. Walzblechprodukt nach einem der Ansprüche 1 bis 8, wobei das Blechprodukt keine metallischen Mantelschichten aufweist.

10. Walzblechprodukt nach einem der Ansprüche 1 bis 9, wobei das Blechprodukt mit einer organischen Beschichtung versehen ist.

11. Walzblechprodukt nach einem der Ansprüche 1 bis 9, wobei das Blechprodukt mittels Blechprägung mit einer Oberflächenstruktur versehen wird.

12. Walzblechprodukt nach einem der Ansprüche 1 bis 11 in Form eines Trapezblechs.

13. Verwendung einer Aluminiumlegierung nach einem der Ansprüche 1 bis 12 zur Verwendung im Außenbereich in der Bauindustrie, Beschilderung oder Dekoration.

14. Verwendung einer Aluminiumlegierung nach einem der Ansprüche 1 bis 12 in Form eines Trapezblechs zur Verwendung im Außenbereich in der Bauindustrie.

## Revendications

1. Produit en tôle d'alliage d'aluminium laminée destiné à l'utilisation en extérieur dans l'industrie du bâtiment, dans lequel l'alliage d'aluminium a la composition suivante, en pourcentage en poids :
| | |
|---|---|
| Si | 1.10 - 1.6 |
| Mg | 0.25 - 0.40 |
| Mn | 0.6 - 1.6 |
| Cu | 0.10 - 0.6 |
| Fe | 0.05 - 0.7 |
| Ti | 0.05 - 0.20 |
| Zn | up to 0.4, |
d'autres éléments et impuretés inévitables, chacune au maximum 0,05 % et au total 0,25 %, le reste étant de l'aluminium.

2. Produit en tôle laminée selon la revendication 1, dans lequel la teneur en Mn est d'au moins 0,70 %, et de préférence d'au moins 0,75 %.

3. Produit en tôle laminée selon la revendication 1 ou 2, dans lequel la teneur en Mn est au plus 1,4 %, et de préférence au plus 1,20 %.

4. Produit en tôle laminée selon l'une quelconque des revendications 1 à 3, dans lequel la teneur en Cu est d'au moins 0,15 %, et de préférence au plus 0,5 %, et de façon plus préférée au plus 0,4 %.

5. Produit en tôle laminée selon l'une quelconque des revendications 1 à 4, dans lequel la teneur en Zn est au plus 0,25 %, et de préférence au plus 0,20 %.

6. Produit en tôle laminée selon l'une quelconque des revendications 1 à 5, dans lequel la teneur en Ti est d'au moins 0,07 %, et de préférence d'au moins 0,08 %.

7. Produit en tôle laminée selon l'une quelconque des revendications 1 à 6, dans lequel la teneur en Ti est au plus 0,17 %, et de préférence au plus 0,15 %.

8. Produit en tôle laminée selon l'une quelconque des revendications 1 à 7, dans lequel la teneur en Si est au plus 1,50 %, et de manière plus préférée au plus 1,45 %.

9. Produit en tôle laminée selon l'une quelconque des revendications 1 à 8, dans lequel le produit en tôle est dépourvu de toute couche de revêtement métallique.

10. Produit en tôle laminée selon l'une quelconque des revendications 1 à 9, dans lequel le produit en tôle est doté d'un revêtement organique.

11. Produit en tôle laminée selon l'une quelconque des revendications 1 à 9, dans lequel le produit en tôle est doté d'une structure de surface via un gaufrage du métal de la tôle.

12. Produit en tôle laminée selon l'une quelconque des revendications 1 à 11, sous la forme d'une tôle trapézoïdale.

13. Utilisation d'un alliage d'aluminium selon l'une quelconque des revendications 1 à 12 destiné à l'utilisation en extérieur dans l'industrie du bâtiment, de la signalisation ou de la décoration.

14. Utilisation d'un alliage d'aluminium selon l'une quelconque des revendications 1 à 12 sous la forme d'une tôle trapézoïdale pour l'utilisation en extérieur dans l'industrie du bâtiment.
